



US008945806B2

(12) **United States Patent**  
Kawakami et al.

(10) **Patent No.:** **US 8,945,806 B2**  
(45) **Date of Patent:** **Feb. 3, 2015**

(54) **ELECTROSTATIC CHARGE IMAGE DEVELOPING TONER, ELECTROSTATIC CHARGE IMAGE DEVELOPER, TONER CARTRIDGE, DEVELOPER CARTRIDGE, PROCESS CARTRIDGE, IMAGE FORMING APPARATUS, AND IMAGE FORMING METHOD**

(75) Inventors: **Eiji Kawakami**, Kanagawa (JP); **Shintaro Anno**, Kanagawa (JP); **Hiroyuki Hamano**, Kanagawa (JP); **Michio Take**, Kanagawa (JP)

(73) Assignee: **Fuji Xerox Co., Ltd.**, Tokyo (JP)

(\*) Notice: Subject to any disclaimer, the term of this patent is extended or adjusted under 35 U.S.C. 154(b) by 15 days.

(21) Appl. No.: **13/557,734**

(22) Filed: **Jul. 25, 2012**

(65) **Prior Publication Data**

US 2013/0252159 A1 Sep. 26, 2013

(30) **Foreign Application Priority Data**

Mar. 23, 2012 (JP) ..... 2012-067654

(51) **Int. Cl.**  
**G03G 9/00** (2006.01)

(52) **U.S. Cl.**  
USPC ..... **430/123.51**; 430/123.41

(58) **Field of Classification Search**  
CPC ..... G03G 9/06; G03G 9/0808; G03G 9/0812;  
G03G 9/09385; G03G 9/08782  
USPC ..... 430/123.51, 123.52, 108.6, 108.7,  
430/123.41  
See application file for complete search history.

(56) **References Cited**

U.S. PATENT DOCUMENTS

5,451,481 A \* 9/1995 Law et al. ..... 430/108.8  
6,190,814 B1 \* 2/2001 Law et al. ..... 430/108.7  
2009/0286176 A1 \* 11/2009 Ohmura et al. ..... 430/107.1

FOREIGN PATENT DOCUMENTS

|    |               |         |
|----|---------------|---------|
| JP | A-06-282096   | 10/1994 |
| JP | A-2005-338690 | 12/2005 |
| JP | A-2008-209489 | 9/2008  |
| JP | A-2008-233736 | 10/2008 |

\* cited by examiner

Primary Examiner — Thorl Chea

(74) **Attorney, Agent, or Firm** — Oliff PLC

(57) **ABSTRACT**

An electrostatic charge image developing toner includes toner particles that contain a colorant, a binder resin and a release agent, and an external additive, in which the external additive contains inorganic particles including an aliphatic alcohol having 5 or more carbon atoms and a melting point of 20° C. or lower on the surfaces thereof.

**12 Claims, No Drawings**

## 1

**ELECTROSTATIC CHARGE IMAGE DEVELOPING TONER, ELECTROSTATIC CHARGE IMAGE DEVELOPER, TONER CARTRIDGE, DEVELOPER CARTRIDGE, PROCESS CARTRIDGE, IMAGE FORMING APPARATUS, AND IMAGE FORMING METHOD**

**CROSS-REFERENCE TO RELATED APPLICATIONS**

This application is based on and claims priority under 35 USC 119 from Japanese Patent Application No. 2012-067654 filed Mar. 23, 2012.

**BACKGROUND**

**1. Technical Field**

The present invention relates to an electrostatic charge image developing toner, an electrostatic charge image developer, a toner cartridge, a developer cartridge, a process cartridge, an image forming apparatus, and an image forming method.

**2. Related Art**

A method of visualizing image information through an electrostatic charge image, such as electrophotography, is now being used in a variety of fields. In electrophotography, an electrostatic charge image (electrostatic latent image) is formed on a photoreceptor (image holding member) through charging and exposure, the electrostatic latent image is developed using a developer including a toner, and visualized through transferring and fixing. The developer that is used in electrophotography includes a two-component developer including a toner and a carrier, and a single-component developer for which a magnetic toner or a non-magnetic toner is singly used, and the toner is manufactured by a kneading and pulverizing manufacturing method in which a thermoplastic resin is melted, kneaded, cooled, then, finely pulverized, and, furthermore, classified together with a pigment, a charge-controlling agent, and a release agent, such as a wax. For the toner, there are cases in which inorganic or organic particles are added to the surfaces of toner particles as necessary in order to improve fluidity or cleaning properties.

**SUMMARY**

According to an aspect of the invention, there is provided an electrostatic charge image developing toner including toner particles that contain a colorant, a binder resin and a release agent, and an external additive, in which the external additive contains inorganic particles including an aliphatic alcohol having 5 or more carbon atoms and a melting point of 20° C. or lower present on the surfaces thereof.

**DETAILED DESCRIPTION**

Hereinafter, exemplary embodiments will be described.

**Electrostatic Charge Image Developing Toner**

The electrostatic charge image developing toner of the exemplary embodiment includes toner particles that contain a colorant, a binder resin and a release agent, and an external additive, in which the external additive contains inorganic particles including an aliphatic alcohol having 5 or more carbon atoms and a melting point of 20° or lower present on the surfaces thereof.

In a developing method in which a two-component developer is used, particularly a magnetic brush method, it is fre-

## 2

quently observed that the toner, that is, toner particles and an external additive accumulate and deform in a cleaning section, so as to remain between a cleaning unit, such as a cleaning blade, and a photoreceptor (image holding member).

5 A phenomenon is displayed in which the sediment that has remained for a long term is fixed to the cleaning blade so as to cause deterioration of cleaning properties, and filming is caused on the photoreceptor such that image defects, such as color streaks due to toner leakage, are caused. In contrast to this, a method in which a silicone oil-treated external additive is added so as to lower the friction coefficient with a photoreceptor is proposed (refer to JP-A-6-282096).

However, the present inventors have observed that, in the toner of the related art as shown in JP-A-6-282096, the silicone oil used for the external additive is coated on the surfaces of the toner particles or the surface of the carrier due to mechanical stress, such as stirring of a developing machine, under conditions of a high temperature and a high humidity, 15 water is absorbed on the surfaces of the toner particles or the carrier due to the hygroscopic properties of the silicone oil so as to form charge-leaking sites, consequently, the charge amount lowers after the toner is placed to stand idle, and image defects, such as fogging, occur.

20 As a result of detailed studies, the inventors have observed that an aliphatic alcohol having 5 or more carbon atoms and a melting point of 20° C. or lower is highly resistant to oxidation deterioration and has a viscosity that does not easily change even under a high temperature and a high humidity, 25 and observed that, when inorganic particles having an aliphatic alcohol that has 5 or more carbon atoms and a melting point of 20° C. or lower present on the surfaces thereof are used as the external additive of the toner, the compound does not easily absorb moisture, occurrence of filming on the photoreceptor is suppressed, and charge stability is excellent even in a case in which the toner is exposed to a high temperature 30 and a high humidity for a long time.

**External Additive**

35 The electrostatic charge developing toner of the exemplary embodiment contains toner particles and an external additive, and the external additive contains inorganic particles having a specific aliphatic alcohol present on the surfaces thereof.

In the inorganic particles having the aliphatic alcohol 40 present on the surfaces thereof, the aliphatic alcohol may be present on at least some of the surfaces of the inorganic particles, but the surfaces of the inorganic particles are coated with the aliphatic alcohol preferably at 50% by area or more, and the surfaces of the inorganic particles are coated with the aliphatic alcohol more preferably at 80% by area or more. The coating amount of the aliphatic alcohol is computed as an average value of 50 or more inorganic particles by dyeing the aliphatic alcohol using a dyeing agent of an organic compound or an aromatic compound, photographing the toner or 45 the inorganic particles, and analyzing the images.

In addition, the aliphatic alcohol is preferably attached to, that is, physically adsorbed on the surfaces of the inorganic particles. With the toner according to the above exemplary embodiment, occurrence of filming is further suppressed 50 even in a case in which the toner is exposed to a high temperature and a high humidity for a long time.

55 It is considered that, since the aliphatic alcohol present on the external additive has a hydrophilic group (OH group) and a hydrophobic group (hydrocarbon chain), the hydrophilic group of the aliphatic alcohol orients in the adsorbed moisture on the surface of the toner or the carrier, and the hydrophobic (hydrocarbon chain) portion migrates outside so that adsorp-

tion of water molecules is hindered, and enlargement of charge-leaking portions is suppressed.

In addition, it is assumed that, in a case in which the aliphatic alcohol is physically adsorbed, some of the aliphatic alcohol is liberated or attaches directly to the carrier, the photoreceptor, or the like from the inorganic particles so that occurrence of filming is further suppressed.

Aliphatic Alcohol Having 5 or More Carbon Atoms and a Melting Point of 20° C. or Lower

The aliphatic alcohol used in the exemplary embodiment is a monovalent alcohol having a saturated chain-type structure with no unsaturated bond and 5 or more carbon atoms, and the melting point of the monovalent alcohol is 20° C. or lower. Any aliphatic alcohol may be used as long as the alcohols satisfies above properties. When the melting point exceeds 20° C., there is a tendency of deterioration of the effect of effectively suppressing occurrence of filming. Meanwhile, the aliphatic alcohol includes alcohols having a straight-chain structure, a branched chain structure, and an alicyclic structure, but alcohols having a straight-chain and a branched chain are preferable, and an alcohol having a branched chain is more preferable.

The number of carbon atoms included in the aliphatic alcohol is preferably 10 or more, more preferably 16 or more, and still more preferably 18 or more. The number of carbon atoms in the aliphatic alcohol is preferably 22 or less, and more preferably 20 or less.

An alkyl group included in the aliphatic alcohol is preferably an alkyl group having a straight-chain or a branched methyl group, and more preferably has a branched methyl group at the end of an alkyl chain apart from a hydroxyl group.

Examples of the aliphatic alcohol include 1-pentanol, 2-pentanol, 1-hexanol, 2-hexanol, 1-octanol, isoctyl alcohol, 2-ethylhexanol, 1-nonanol, 1-decanol, isostearyl alcohol, cyclopentanol and cyclooctanol, and isostearyl alcohol is more preferable.

The electrostatic charge image developing toner of the exemplary embodiment contains toner particles including at least a colorant, a binder resin and a release agent, and an external additive having an aliphatic alcohol having 5 or more carbon atoms and a melting point of 20° C. or lower present on the surface thereof so that image defects caused by photoreceptor filming may be suppressed, and background fogging due to charge leakage may be reduced under a high temperature and a high humidity.

The mechanism is not clear, but it is assumed that, probably, since the aliphatic alcohol present on the external additive has a hydrophilic group (OH group) and a hydrophobic group (hydrocarbon chain), the hydrophilic group of the aliphatic alcohol orients in the adsorbed moisture on the surface of the toner or the carrier, and the hydrophobic (hydrocarbon chain) portion migrates outside so that adsorption of water molecules is hindered, and enlargement of charge-leaking portions is suppressed.

It is assumed that, for aliphatic alcohols having up to 4 carbon atoms, since the hydrocarbon chains are short, the hydrophobicity is not sufficient, aliphatic alcohol molecules may not orient with respect to adsorbed moisture molecules on the surfaces of the toner and the carrier, and enlargement of the charge-leaking portions may not be suppressed.

In addition, the melting point of the aliphatic alcohol used for the exemplary embodiment should be 20° C. or lower. It is assumed that, when the melting point is higher than 20° C., since the aliphatic alcohol becomes solid under a high temperature and a high humidity, the aliphatic alcohol molecules may not orient with respect to the adsorbed moisture on the

surfaces of the toner and the carrier, and enlargement of the charge-leaking portions may not be suppressed.

#### Inorganic Particles

The inorganic particles having the aliphatic alcohol present on the surfaces thereof are not particularly limited, and well-known inorganic particles may be used as the external additive of the toner. Examples thereof include silica, alumina, titania (titanium oxide, meta titanium oxide, and the like), cerium oxide, zirconia, calcium carbonate, magnesium carbonate, calcium phosphate, carbon black, and the like.

Among the above, silica particles or titanium oxide particles are preferable, and silica particles are particularly preferable.

The silica particles include silica particles, such as fumed silica, colloidal silica, and silica gel.

In addition, the inorganic particles may not only have the aliphatic alcohol present on the surfaces thereof but also, for example, the surfaces may be treated using a silica coupling agent or the like which will be described below.

The volume average primary particle diameter of the inorganic particles is preferably from 3 nm to 500 nm, more preferably from 7 nm to 300 nm, still more preferably from 10 nm to 200 nm, and particularly preferably from 10 nm to 130 nm. Within the above range, the migratory properties of the aliphatic alcohol into the carrier, the photoreceptor, or the like are excellent, and occurrence of filming is further suppressed.

The volume average primary particle diameter of the inorganic particles is preferably measured using LS13 320 (manufactured by Beckman Coulter, Inc.).

In addition, in the toner of the exemplary embodiment, the volume average primary particle diameter of the inorganic particles having the aliphatic alcohol present on the surfaces thereof is preferably larger than the volume average primary particle diameter of the external additive other than the inorganic particles.

In the toner of the exemplary embodiment, the content of the inorganic particles having the aliphatic alcohol present on the surfaces thereof is not particularly limited, but is preferably from 0.3% by weight to 10% by weight, more preferably from 0.5% by weight to 5% by weight, and still more preferably from 0.8% by weight to 2.0% by weight of the total weight of the toner.

Method of Manufacturing the Inorganic Particles Having the Aliphatic Alcohol Present on the Surface Thereof (Surface Treatment Method)

A method of manufacturing the inorganic particles having the aliphatic alcohol present on the surface thereof is not particularly limited, and a well-known method may be used. In addition, even in a state in which the aliphatic alcohol is physically adsorbed to the surfaces of the inorganic particles, the effects of the invention are sufficiently exhibited. A chemical treatment, such as baking through heating, may not be carried out.

Examples of the physical adsorption treatment method include a method of drying through a spray drying method in which the aliphatic alcohol or a liquid including the aliphatic alcohol is sprayed to the inorganic particles floating in a gaseous phase or the like, a method in which the inorganic particles are immersed in a solution containing the aliphatic alcohol and dried, and the like. In addition, the inorganic particles that have undergone the physical adsorption treatment may be heated, and the surfaces of the inorganic particles may be chemically treated using the aliphatic alcohol.

In the toner of the exemplary embodiment, the amount of the aliphatic alcohol treated on the inorganic particles (the content of the aliphatic alcohol in the toner) is preferably 0.16% by weight or more, and more preferably 0.2% by

weight or more, and preferably 5% by weight or less, and more preferably 1.0% by weight or less of the total weight of the toner. Within the above range, the filming suppression effect is further exhibited.

Examples of a method of externally adding the external additive to the toner of the exemplary embodiment include a method in which toner particles and the external additive are mixed using a Henschel mixer, a V blender, or the like so as to manufacture the inorganic particles. In addition, in a case in which toner particles are manufactured in a wet manner, it is also possible to externally add the external additive in a wet manner.

In addition, a method is also included in which, after the inorganic particles are externally added to the toner particles, the aliphatic alcohol or a liquid including the aliphatic alcohol is added, and the mixture is mixed using a Henschel mixer, a V blender, or the like.

Among the above, the method of manufacturing the inorganic particles through a physical adsorption treatment is preferable as the method of manufacturing the inorganic particles having the aliphatic alcohol present on the surface thereof.

#### Other External Additives

The toner of the exemplary embodiment may include external additives other than the inorganic particles having the aliphatic alcohol present on the surface thereof (also referred to as "other external additives").

The content of other external additives in the toner of the exemplary embodiment may be smaller than that of the inorganic particles having the aliphatic alcohol present on the surface thereof.

Examples of other external additives include inorganic particles described above and resin particles of a vinyl resin, a polyester resin, a silicone resin, and the like.

Regarding the inorganic particles in other external additives, the surfaces thereof are preferably hydrophobized in advance. The hydrophobization treatment is more effective for not only improvement of the powder fluidity of the toner, but also the environment dependence of charge and carrier contamination resistance.

The hydrophobization treatment is carried out by immersing the inorganic particles in a hydrophobizing agent, or the like. The hydrophobizing agent is not particularly limited, and examples thereof include a silane coupling agent, a titanate coupling agent, an aluminum coupling agent, and the like. The hydrophobizing agent may be used singly, or two or more kinds thereof may be jointly used. Among the above, a silane coupling agent is preferably included.

Examples of the silane coupling agent that may be used include any type of chlorosilane, alkoxy silane, silazane, special silylation agents.

Specific examples include methyltrichlorosilane, dimethylchlorosilane, trimethylchlorosilane, phenyltrichlorosilane, diphenylchlorosilane, tetramethoxy silane, methyltrimethoxysilane, dimethyldimethoxysilane, phenyltrimethoxysilane, diphenyldimethoxysilane, tetraethoxysilane, methyltriethoxysilane, dimethyldiethoxysilane, phenyltriethoxysilane, diphenyldiethoxysilane, isobutyltriethoxysilane, decyltrimethoxysilane, hexamethyldisilazane, N,O-(bistrimethylsilyl)acetamide, N,N-(trimethylsilyl)urea, tert-butyldimethylchlorosilane, vinyltrichlorosilane, vinyltrimethoxysilane, vinyltriethoxysilane,  $\gamma$ -methacryloxypropyltrimethoxysilane,  $\beta$ -(3,4-epoxypropyl)ethyltrimethoxysilane,  $\gamma$ -glycidoxypropyltrimethoxysilane,  $\gamma$ -mercaptopropyltrimethoxysilane,  $\gamma$ -chloropropyl trimethoxysilane, and the like.

The amount of the hydrophobizing agent changes by the kind of the inorganic particles and the like, and may not be generally specified. However, the amount is preferably from 1 part by weight to 50 parts by weight, and more preferably from 5 parts by weight to 20 parts by weight with respect to 100 parts by weight of the inorganic particles. Meanwhile, in the exemplary embodiment, a commercially available product is also preferably used as the hydrophobic silica particles.

The average primary particle diameter of other external additives is preferably from 3 nm to 500 nm, more preferably from 5 nm to 100 nm, still more preferably from 5 nm to 50 nm, and particularly preferably from 5 nm to 40 nm.

#### Toner Particles

The electrostatic charge image developing toner of the exemplary embodiment contains toner particles containing a colorant, a binder resin, and a release agent. In addition, the toner particles may further contain a well-known additive, such as a charge-controlling agent.

#### Binder Resin

The binder resin includes polyolefin resin, such as polyethylene and polypropylene, styrene resin mainly including polystyrene, poly( $\alpha$ -methylstyrene), or the like, (meth)acryl resin mainly including polymethyl methacrylate, polyacrylonitrile, or the like, styrene-(meth) acryl copolymer resin, polyamide resin, polycarbonate resin, polyether resin, polyester resin, and copolymer resin thereof, but styrene resin, (meth)acryl resin, styrene-(meth)acryl copolymer resin, or polyester resin is preferable from the viewpoint of charge stability and developing durability when being used for the electrostatic charge image developing toner.

The binder resin preferably contains a polyester resin, and more preferably contain an amorphous (non-crystalline) polyester resin from the viewpoint of low-temperature fixing properties.

The polyester resin is obtained through, for example, condensation polymerization of mainly a polyvalent carboxylic acid and a polyol.

Examples of the polyvalent carboxylic acid include aromatic carboxylic acids, such as terephthalic acid, isophthalic acid, phthalic anhydride, trimellitic anhydride, pyromellitic acid, and naphthalenedicarboxylic acid; aliphatic carboxylic acids, such as maleic anhydride, fumaric acid, succinic acid, alkenyl succinic anhydride, and adipic acid; alicyclic carboxylic acids, such as cyclohexane dicarboxylic acid; lower alkyl esters or acid anhydrides thereof. Meanwhile, the lower alkyl refers to a straight-chain, branched or cyclic alkyl group having from 1 to 8 carbon atoms. The polyvalent carboxylic acid may be used singly, or two or more kinds thereof may be jointly used. Among the polyvalent carboxylic acids, the aromatic carboxylic acid is preferably used. In addition, a tri- or higher valent carboxylic acid (trimellitic acid, acid anhydride thereof, or the like) is preferably used jointly with a dicarboxylic acid in order to have a crosslinking structure or a branched structure for the purpose of securing favorable fixing properties.

Examples of the polyvalent carboxylic acid used to obtain the amorphous polyester resin include aromatic dicarboxylic acids, such as phthalic acid, isophthalic acid, terephthalic acid, naphthalene-2,6-dicarboxylic acid, 1,4-phenylene diacetate, and 1,4-cyclohexanedicarboxylic acid; dicarboxylic acids having alicyclic hydrocarbon group, and the like, and also includes acid anhydrides and lower alkyl esters thereof.

Examples of the polyol include aliphatic diols, such as ethylene glycol, diethylene glycol, triethylene glycol, propylene glycol, butanediol, hexanediol, neopentyl glycol, and glycerin; alicyclic diols, such as cyclohexanediol, cyclohexanedimethanol, and hydrogenated bisphenol A; aromatic

diols, such as ethylene oxide adducts of bisphenol A and propylene oxide adducts of bisphenol A. The polyol may be used singly, or two or more kinds thereof may be jointly used.

Preferable examples of the polyol used to obtain the amorphous polyester include aliphatic, alicyclic, and aromatic polyols, and specific examples thereof include 1,4-cyclohexanediol, 1,4-cyclohexanediethanol, alkylene oxide adducts of bisphenol A, alkylene oxide adducts of bisphenol Z, alkylene oxide adducts of hydrogen-added bisphenol A, and the like. Among the above, an alkylene oxide adduct of bisphenol A may be preferably used, and an adduct of 2 moles of ethylene oxide of bisphenol A and an adduct of 2 moles of propylene oxide of bisphenol A may be more preferably used.

In addition, a tri- or higher valent alcohol (for example, glycerine, trimethylol propane, pentaerythritol, or the like) may be used jointly with a diol in order to have a crosslinking structure or a branched structure for the purpose of securing more favorable fixing properties.

The glass transition temperature (hereinafter sometimes abbreviated to be "Tg") of the amorphous polyester resin is preferably from 50° C. to 80° C., and more preferably from 50° C. to 70° C. When Tg is 80° C. or lower, the low-temperature fixing properties are excellent, which is preferable. In addition, when Tg is 50° C. or higher, the heat preservation resistance is excellent, and the preservation properties of fixed images are excellent, which are preferable.

The acid value of the amorphous polyester resin is preferably from 5 mg KOH/g to 25 mg KOH/g, and more preferably from 6 mg KOH/g to 23 mg KOH/g. When the acid value is 5 mg KOH/g or more, the affinity of the toner to paper is favorable, and the charging properties are also favorable. In addition, in a case in which the toner is manufactured by an emulsion and aggregation method described below, emulsified particles are easily manufactured, the large acceleration of the aggregation rate during aggregation process or the shape change rate during coalescence process in the emulsion and aggregation method is suppressed, and particle sizes and shapes are easily controlled. In addition, when the acid value of the amorphous polyester resin is 25 mg KOH/g or less, the environment dependence of charging is not adversely influenced. In addition, the large deceleration of the aggregation rate during aggregation process or the shape change rate during coalescence process in manufacture of the toner by the emulsion and aggregation method is suppressed, and deterioration of the productivity is prevented.

For the amorphous polyester resin, when molecular weights are measured by the gel permeation chromatography (GPC) of tetrahydrofuran (THF) soluble, the weight average molecular weight (Mw) is preferably from 5,000 to 1,000,000, and more preferably from 7,000 to 500,000, the number average molecular weight (Mn) is preferably from 2,000 to 100,000, and the molecular weight distribution Mw/Mn is preferably from 1.5 to 100, and more preferably from 2 to 60.

When the molecular weight and molecular weight distribution of the amorphous polyester resin are within the above ranges, excellent fixed image strength may be obtained without impairing the low-temperature fixing properties, which is preferable.

In the exemplary embodiment, the toner particles may include a crystalline polyester resin.

The crystalline polyester resin is compatible with the amorphous polyester resin during melting so as to largely lower the toner viscosity, thereby obtaining a toner having more favorable low-temperature fixing properties. In addition, among the crystalline polyester resins, since many aromatic crystalline polyester resins are generally melted at a higher temperature than the melting temperature range

described below, the crystalline polyester resin is more preferably an aliphatic crystalline polyester resin in a case in which the toner particles includes the crystalline polyester resin.

In the exemplary embodiment, the content of the crystalline polyester resin in the toner particles is preferably from 2% by weight to 30% by weight, and more preferably from 4% by weight to 25% by weight. When the content is 2% by weight or more, it is possible to decrease the viscosity of the amorphous polyester resin during melting, and the low-temperature fixing properties may be easily improved. In addition, when the content is 30% by weight or less, deterioration of the charging properties of the toner which is caused by the presence of the crystalline polyester resin is prevented, and, furthermore, high image strength may be easily obtained after the toner is fixed to a recording medium.

The melting temperature of the crystalline polyester resin is preferably in a range of 50° C. to 90° C., more preferably in a range of 55° C. to 90° C., and still more preferably in a range of 60° C. to 90° C. When the melting temperature is 50° C. or higher, the preservation properties of the toner or the preservation properties of the fixed toner images are excellent. In addition, when the melting temperature is 90° C. or lower, the low-temperature fixing properties improve.

On the other hand, the glass transition temperature (Tg) of the amorphous polyester resin is preferably 30° C. or higher, more preferably from 30° C. to 100° C., and still more preferably from 50° C. to 80° C. Within the above ranges, since the amorphous polyester resin is in a glass state while being used, toner particles are not aggregated due to heat or pressure applied during formation of an image, and a stable image forming ability may be obtained for a long time without the toner particles being attached to and accumulated in a machine.

The glass transition temperature of the resin may be measured by a well-known method, for example, the method described in ASTM D3418-82 (DSC method).

The melting point of the crystalline resin is measured using a differential scanning calorimeter (DSC), and may be obtained as a melting peak temperature of input compensation differential scanning calorimetry shown in JIS K-7121 when measurement is carried out at a temperature-increase rate of 10° C./min from room temperature to 150° C.

Meanwhile, the "crystalline" as shown in the crystalline resin indicates that the resin does not show stepwise endothermic change, but has a clear endothermic peak, and specifically means that the half-value width of the endothermic peak is 15° C. or less when measurement is carried out at a temperature-increase rate of 10° C./min.

On the other hand, a resin for which the half-value width of the endothermic peak exceeds 15° C. and a resin for which a clear endothermic peak is not observed indicate that they are not crystalline (amorphous). The glass transition temperature of the amorphous resin is measured by DSC based on ASTM D3418 using a differential scanning calorimeter (DSC-50 manufactured by Shimadzu Corporation) having an automatic tangential treatment system. The measurement conditions are as follows.

Sample: 3 mg to 15 mg, preferably 5 mg to 10 mg  
Measurement method: the sample is put in an aluminum pan, and an empty aluminum pan is used as a reference.

Temperature Curve: Temperature Increase I (20° C. to 180° C., Temperature-Increase Rate 10° C./min)

In the above temperature curve, the glass transition temperature is measured from the endothermic curve measured during temperature increase.

The glass transition temperature is a temperature at which the differential value of the endothermic curve becomes the maximum.

In addition, in a case in which the crystalline polyester resin is a polymer in which other components are copolymerized with the main chain, and the content of the other components is less than 50% by weight, the copolymer is also termed a crystalline polyester.

Examples of the acid component used for synthesis of the crystalline polyester resin include a variety of polyvalent carboxylic acids, but a dicarboxylic acid is preferable, and a straight-chain-type aliphatic dicarboxylic acid is more preferable.

Examples thereof include oxalic acid, malonic acid, succinic acid, glutaric acid, adipic acid, pimelic acid, suberic acid, azelaic acid, sebatic acid, 1,9-nonane dicarboxylic acid, 1,10-decanedicarboxylic acid, 1,11-undecanedicarboxylic acid, 1,12-dodecanedicarboxylic acid, 1,13-tridecanedicarboxylic acid, 1,14-tetradecane dicarboxylic acid, 1,16-hexadecanedicarboxylic acid, 1,18-octadecanedicarboxylic acid, and the like, lower alkyl esters or acid anhydrides thereof, but the acid component is not limited thereto. Among the above, adipic acid, sebatic acid, and 1,10-decanedicarboxylic acid are preferable in consideration of easy procurement.

In addition, as the acid component used for synthesis of the crystalline polyester resin, dicarboxylic acid having an ethylenic unsaturated bond or dicarboxylic acid having a sulfonic acid group may be used.

Aliphatic diols are preferable as the alcohol component used for synthesis of the crystalline polyester resin, and examples thereof include ethylene glycol, 1,3-propanediol, 1,4-butanediol, 1,5-pentanediol, 1,6-hexanediol, 1,7-heptanediol, 1,8-octanediol, 1,9-nonanediol, 1,10-decanediol, 1,11-dodecanediol, 1,12-undecanediol, 1,13-tridecanediol, 1,14-tetradecanediol, 1,18-octadecanediol, 1,20-eicosanediol, and the like, but the alcohol component is not limited thereto. Among the above, 1,4-butanediol, 1,6-hexanediol, 1,8-octanediol, 1,9-nonanediol, and 1,10-decanediol are preferable in consideration of easy procurement and the cost.

The molecular weight (weight average molecular weight;  $M_w$ ) of the crystalline polyester resin is preferably from 8,000 to 40,000, and more preferably from 10,000 to 30,000 from the viewpoints of the manufacturability of the resin, fine dispersion of the toner during manufacturing, and the compatibility during melting. When the weight average molecular weight is 8,000 or more, decreasing of the electric resistance of the crystalline polyester resin is suppressed, and therefore deterioration of the charging properties is prevented. In addition, when the weight average molecular weight is 40,000 or less, costs for resin synthesis are suppressed, and deterioration of the sharp melting properties is prevented, and therefore the low-temperature fixing properties are not adversely influenced.

In the exemplary embodiment, the molecular weight of the polyester resin is measured and computed by gel permeation chromatography (GPC). Specifically, for the measurement, a HLC-8120 manufactured by Tosoh Corporation is used as the GPC, a TSKgel Super HM-M (15 cm) manufactured by Tosoh Corporation is used as the column, and a polyester resin is measured with the THF solvent. Next, the molecular weight of the polyester resin is computed using a molecular weight calibration curve prepared from a monodisperse polystyrene standard sample.

A method of manufacturing the polyester resin is not particularly limited, and the polyester resin may be manufac-

tured by a general polyester polymerization method in which the acid component and the alcohol component are reacted with each other. For example, any of direct condensation polymerization, an ester exchange method, and the like are selected depending on the kind of a monomer so as to manufacture the polyester resin. When the acid component and the alcohol component are reacted with each other, since the molar ratio (the acid component/the alcohol component) varies with reaction conditions and the like, it is not possible to specify a comprehensive molar ratio, but the molar ratio is, generally, preferably approximately 1/1 in order to increase the molecular weight.

The catalyst that may be used to manufacture the polyester resin includes alkali metal compounds of sodium, lithium, and the like; alkaline earth metal compounds of magnesium, calcium, and the like, metal compounds of zinc, manganese, antimony, titanium, tin, zirconium, germanium, and the like; phosphite compounds, phosphate compounds, amine compounds, and the like.

10 A styrene resin and a (meth) acryl resin, particularly, a styrene-(meth) acryl copolymer resin is useful as the binder resin in the exemplary embodiment.

Latex having a copolymer obtained by polymerizing a monomer mixture including 60 parts by weight to 90 parts by 15 weight of a vinyl aromatic monomer (styrene monomer), 10 parts by weight to 40 parts by weight of ethylenic unsaturated carboxylic acid ester monomer ((meth) acrylic acid ester monomer), and 1 part by weight to 3 parts by weight of an ethylenic unsaturated monomer, which is dispersed and stabilized using a surfactant, may be preferably used as the 20 binder resin component.

The glass transition temperature of the copolymer is preferably from 50° C. to 70° C.

Hereinafter, polymerizable monomers that compose the 25 copolymer resin will be described.

Examples of the styrene monomer include alkyl-substituted styrene having an alkyl chain, such as styrene,  $\alpha$ -methyl styrene, vinyl naphthalene, 2-methyl styrene, 3-methyl styrene, 4-methyl styrene, 2-ethyl styrene, 3-ethyl styrene, and 30 4-ethyl styrene; halogen-substituted styrene, such as 2-chlorostyrene, 3-chlorostyrene, and 4-chlorostyrene; fluorine-substituted styrene, such as 4-fluorostyrene and 2,5-difluorostyrene; and the like. Among the above, styrene is preferable as the styrene monomer.

As the (meth)acrylate ester monomer, there are n-methyl (meth)acrylate, n-ethyl (meth)acrylate, n-propyl (meth)acrylate, n-butyl (meth)acrylate, n-pentyl (meth)acrylate, n-hexyl (meth)acrylate, n-heptyl (meth)acrylate, n-octyl (meth)acrylate, n-decyl (meth)acrylate, n-dodecyl (meth)acrylate, n-lauryl (meth)acrylate, n-tetradecyl (meth)acrylate, n-hexadecyl (meth)acrylate, n-octadecyl (meth)acrylate, isopropyl (meth)acrylate, isobutyl (meth)acrylate, t-butyl (meth)acrylate, isopentyl (meth)acrylate, amyl (meth)acrylate, neopentyl (meth)acrylate, isohexyl (meth)acrylate, isoheptyl (meth) 45 acrylate, isoctyl (meth)acrylate, 2-ethylhexyl (meth)acrylate, phenyl (meth)acrylate, biphenyl (meth)acrylate, diphenylethyl (meth)acrylate, t-butylphenyl (meth)acrylate, terphenyl (meth)acrylate, cyclohexyl (meth)acrylate, t-butyl cyclohexyl (meth)acrylate, dimethylaminoethyl (meth)acrylate, diethylaminoethyl (meth)acrylate, methoxyethyl (meth)acrylate, 50 2-hydroxyethyl (meth)acrylate,  $\beta$ -carboxyethyl (meth)acrylate, (meth)acrylonitrile, (meth)acrylamide, and the like. Among the above, n-butyl acrylate is preferable as the (meth)acrylate ester monomer.

55 The ethylenic unsaturated acid monomer is an ethylenic unsaturated monomer containing an acidic group, such as a carboxyl group, a sulfonic acid group, or an acid anhydride. 60

## 11

In a case in which a carboxyl group is to be contained in the styrene resin, the (meth)acryl resin, and the styrene-(meth)acryl copolymer resin, it is possible to obtain the resin by copolymerizing polymerizable monomers having a carboxylic group.

Specific examples of the carboxylic group-containing polymerizable monomer include acrylic acid, aconic acid, atropic acid, arylmalonic acid, angelic acid, isocrotonic acid, itaconic acid, 10-undecenic acid, elaidic acid, erucic acid, oleic acid, o-carboxycinnamic acid, crotonic acid, chloroacrylic acid, chloroisocrotonic acid, chlorocrotonic acid, chlorofumaric acid, chloromaleic acid, cinnamic acid, cyclohexenedicarboxylic acid, citraconic acid, hydroxyl cinnamic acid, dihydroxycinnamic acid, tiglic acid, nitro cinnamic acid, vinyl acetate, phenyl cinnamic acid, 4-phenyl-3-butenoic acid, ferulic acid, fumaric acid, brassidic acid, 2-(2-furyl)acrylate, bromocinnamic acid, bromo fumaric acid, bromo maleic acid, benzylidene malonic acid, benzoyl acrylate, 4-pentenoic acid, maleic acid, mesaconic acid, methacrylic acid, methyl cinnamic acid, methoxy cinnamic acid, and the like. Among the above, acrylic acid, methacrylic acid, maleic acid, cinnamic acid, and fumaric acid are preferable and acrylic acid is more preferable in terms of easiness of a polymer-forming reaction.

A chain transfer agent may be used when the binder resin is polymerized.

The chain transfer agent is not particularly limited, and a compound having a thiol component may be used. Specifically, alkyl mercaptans, such as hexyl mercaptan, heptyl mercaptan, octyl mercaptan, nonyl mercaptan, decyl mercaptan, and dodecyl mercaptan, are preferable. They are preferable particularly because the molecular weight distribution is narrow, and thus the preservation properties of the toner at a high temperature become favorable.

A crosslinking agent may be added to the binder resin as necessary. The crosslinking agent is typically a multifunctional monomer having 2 or more ethylenic unsaturated groups in the molecule.

Specific examples of the crosslinking agent include aromatic polyvinyl compounds, such as divinylbenzene and divinylnaphthalene; polyvinyl esters of aromatic polyvalent carboxylic acid, such as divinyl phthalate, divinyl isophthalate, divinyl terephthalate, divinyl homophthalate, divinyl/trivinyl trimesate, divinyl naphthalene dicarboxylate, and divinyl biphenylcarboxylate; divinyl esters of nitrogen-containing aromatic compounds, such as divinyl pyridine dicarboxylate; vinyl esters of unsaturated heterocyclic compound carboxylic acids, such as vinyl pyromucate, vinyl furan carboxylate, vinyl pyrrole-2-carboxylate, and vinyl thiophene carboxylate; (meth)acrylates of linear polyols, such as butanediol methacrylate, hexanediol acrylate, octanediol methacrylate, decanediol acrylate, and dodecanediol methacrylate; branched and substituted polyol (meth)acrylates, such as neopentyl glycol dimethacrylate and 2-hydroxy-1,3-diacryloxy propane; polyethylene glycol di(meth)acrylate, polypropylene polyethylene glycol di(meth)acrylates; and polyvalent polyvinyl carboxylates, such as divinyl succinate, divinyl fumarate, vinyl/divinyl maleate, divinyl diglycolate, vinyl/divinyl itaconate, divinyl acetone dicarboxylate, divinyl glutarate, divinyl 3,3'-thiodipropionate, divinyl/trivinyl trans-aconate, divinyl adipate, divinyl pimelate, divinyl suberate, divinyl azelate, divinyl sebacate, dodecane diacid divinyl, divinyl brassylate, and the like.

In the exemplary embodiment, the crosslinking agent may be used singly, or two or more kinds may be jointly used.

The preferable content of the crosslinking agent is preferably in a range of 0.05% by weight to 5% by weight, and more

## 12

preferably in a range of 0.1% by weight to 1.0% by weight of the total amount of the polymerizable monomer.

Among the binder resins, binder resins that may be manufactured through radical polymerization of polymerizable monomers may be polymerized using a radical polymerization initiator.

The radical polymerization initiator is not particularly limited, and specific examples thereof include peroxides, such as hydrogen peroxide, acetyl peroxide, cumyl peroxide, tert-butyl peroxide, propionyl peroxide, benzoyl peroxide, chlorobenzoyl peroxide, dichlorobenzoyl peroxide, bromomethyl benzoyl peroxide, lauroyl peroxide, ammonium persulfate, sodium persulfate, potassium persulfate, peroxy carbonate diisopropyl, tetralin hydroperoxide, 1-phenyl-2-methylpropyl-1-hydroperoxide, pertriphenyl acetate-tert-butyl hydroperoxide, tert-butyl performate, tert-butyl peracetate, tert-butyl perbenzoate, tert-butyl perphenylacetate, tert-butyl permethoxyacetate, and tert-butyl perN-(3-toluoyl)carbamate; azo compounds such as 2,2'-azobisisopropane, 2,2'-dichloro-2,2'-azobisisopropane, 1,1'-azo(methyl ethyl)diacetate, 2,2'-azobis(2-amidinopropane)hydrochloride, 2,2'-azobis(2-amidinopropane)nitrate, 2,2'-azobisisobutane, 2,2'-azobisisobutylamide, 2,2'-azobisisobutyronitrile, methyl 2,2'-azobis-2-methylpropionate, 2,2'-dichloro-2,2'-azobisisobutane, 2,2'-azobis-2-methylbutyronitrile, dimethyl 2,2'-azobisisobutyl, 1,1'-azobis(sodium 1-methylbutyronitrile-3-sulfonate), 2-(4-methylphenylazo)-2-methylmalonodinitrile, 4,4'-azobis-4-cyanovaleic acid, 3,5-dihydroxymethylphenylazo-2-methylmalonodinitrile, 2-(4-bromophenylazo)-2-allylmalonodinitrile, 2,2'-azobis-2-methylvaleronitrile, dimethyl 4,4'-azobis-4-cyanovaleate, 2,2'-azobis-2,4-dimethylvaleronitrile, 1,1'-azobiscyclohexanenitrile, 2,2'-azobis-2-propylbutyronitrile, 1,1'-azobis-1-chlorophenylethane, 1,1'-azobis-1-cyclohexanecarbonitrile, 1,1'-azobis-1-cycloheptanenitrile, 1,1'-azobis-1-phenylethane, 1,1'-azobiscumene, ethyl 4-nitrophenylazobenzylcyanoacetate, phenyl azodiphenyl methane, phenyl azotriphenyl methane, 4-nitrophenyl azotriphenyl methane, 1,1'-azobis-1,2-diphenyl ethane, poly(bisphenol A-4,4'-azobis-4-cyanopentanoate) and poly(tetraethylene glycol-2,2'-azobisisobutyrate); 1,4-bis(pentaethylene)-2-tetrazene, 1,4-dimethoxycarbonyl-1,4-diphenyl-2-tetrazene, and the like.

In addition, examples of the crystalline vinyl resin include vinyl resins using (meth)acrylate esters of long-chain alkyl or alkenyl, such as amyl(meth)acrylate, hexyl(meth)acrylate, heptyl(meth)acrylate, octyl(meth)acrylate, nonyl(meth)acrylate, decyl(meth)acrylate, undecyl(meth)acrylate, tridecyl(meth)acrylate, myristyl(meth)acrylate, cetyl(meth)acrylate, stearyl(meth)acrylate, oleyl(meth)acrylate and behenyl(meth)acrylate. Meanwhile, in the present specification, the term "(meth)acryl" means inclusion of any or both of "acryl" and "methacryl".

In addition, the weight average molecular weight of the addition polymerization-type resin, such as styrene resin and (meth) acryl resin, is preferably from 5,000 to 50,000 and more preferably from 7,000 to 35,000. When the weight average molecular weight is 5,000 or more, the cohesive force as the binder resin is favorable, and the hot offset properties do not degrade. In addition, when the weight average molecular weight is 50,000 or less, favorable hot offset properties and a favorable lowest fixing temperature may be obtained, the time or temperature necessary for condensation polymerization are appropriate, and manufacturing efficiency is favorable.

Meanwhile, the weight average molecular weight of the binder resin may be measured through, for example, gel permeation chromatography (GPC) and the like.

The content of the binder resin in the toner of the exemplary embodiment is not particularly limited, but is preferably from 10% by weight to 95% by weight, more preferably from 25% by weight to 90% by weight, and still more preferably from 45% by weight to 85% by weight with respect to the total weight, of the toner. Within the above ranges, fixing properties, charge characteristics, and the like are excellent.

#### Colorant

The toner particles contain a colorant.

Examples of the colorant that may be used for the toner of the exemplary embodiment include one kind or a combination of two or more kinds of magnetic powder of magnetite, ferrite, and the like; a variety of pigments, such as carbon black, lampblack, chrome yellow, hanza yellow, benzidine yellow, threne yellow, quinoline yellow, permanent orange GTR, pyrazolone orange, vulcan orange, Watchung red, permanent red, brilliant carmine 3B, brilliant carmine 6B, DuPont oil red, pyrazolone red, lithol red, rhodamine B lake, lake red C, rose Bengal, aniline blue, chalco oil blue, methylene blue chloride, phthalocyanine blue, phthalocyanine green, and malachite green oxalate; a variety of dyes based on acridine, xanthene, azo, benzoquinone, azine, anthraquinone, thioindigo, dioxazine, thiazine, azomethine, indigo, phthalocyanine, aniline black, polymethine, triphenyl methane, diphenyl methane, and thiazole.

In addition, examples thereof include C.I. Pigment Red 48:1, C.I. Pigment Red 122, C.I. Pigment 57:1, C.I. Pigment Yellow 97, C.I. Pigment Yellow 17, C.I. Pigment Blue 15:1, C.I. Pigment Blue 15:3, and the like.

The content of the colorant in the toner particles is preferably in a range of 1 part by weight to 30 parts by weight with respect to 100 parts by weight of the binder resin in the toner particles. In addition, it is also effective to use a surface-treated colorant or a pigment dispersing agent as necessary. A toner having a variety of colors, such as a yellow toner, a magenta toner, a cyan toner, and a black toner, may be obtained by appropriately selecting the kinds of the colorant.

#### Release Agent

The toner particles contain a release agent.

The release agent used in the exemplary embodiment is not particularly limited, a well-known release agent may be used, and the following waxes are preferable.

Examples of the waxes include a paraffin wax and derivatives thereof, a montan wax and derivatives thereof, a micro-crystalline wax and derivatives thereof, a Fischer Tropsch wax and derivatives thereof, a polyolefin wax and derivatives thereof, and the like. The derivatives include oxides, polymers with vinyl monomers, and graft modification products. Additionally, an alcohol, an aliphatic acid, a plant wax, an animal wax, a mineral wax, an ester wax, an acid amide, and the like may also be used.

The wax used as the release agent is melted at any of temperature of 70° C. to 140° C., and preferably shows a melting viscosity of 1 centipoise to 200 centipoises, and more preferably a melting viscosity of 1 centipoise to 100 centipoises. When the wax is melted at 70° C. or higher, the change temperature of the wax is sufficiently high, and the blocking resistance and the developing properties when the temperature inside a copying machine is increased are excellent. When the wax is melted at 140° C. or lower, the change temperature of the wax is sufficiently low, it is not necessary to carry out fixing at a high temperature, and energy saving properties are excellent. In addition, when the melting viscosity is 200 centipoises or less, the degree of ejection from the toner is appropriate, and the fixing peeling properties are excellent.

In the toner of the exemplary embodiment, the release agent is selected from the viewpoints of fixing properties, toner blocking properties, toner strength, and the like. The added amount of the release agent is not particularly limited, but is preferably in a range of 2 parts by weight to 20 parts by weight with respect to 100 parts by weight of the bidding resin included in the toner particles.

#### Other Additives

In addition to the above components, a variety of components, such as an internal additive and a charge-controlling agent, may be further added to the coloring particles as necessary.

Examples of the internal additive include magnetic articles, such as metals, such as ferrite, magnetite, reduced iron, cobalt, nickel, and manganese, alloys, and compounds including the metals.

Examples of the charge-controlling agent include quaternary ammonium salt compounds, nigrone compounds, dyes including a complex, such as aluminum, iron, or chromium, triphenyl methane pigments, and the like.

The toner particles used in the exemplary embodiment is not particularly limited by the manufacturing method, and may be manufactured by a well-known method. Specific examples include the following methods.

The toner particles may be manufactured by, for example, a kneading and pulverizing method in which the binder resin, the colorant, the release agent, the charge-controlling agent as necessary, and the like are kneaded, pulverized, and classified; a method in which the shapes of particles obtained by the kneading and pulverizing method are changed through a mechanical impulsive force or heat energy; an emulsion and aggregation method in which a dispersion liquid obtained by emulsifying and dispersing the binder resin and a dispersion liquid of the colorant, the release agent, the charge-controlling agent as necessary, and the like are mixed, aggregated, heated, and coalesced so as to obtain toner particles; an emulsion polymerization aggregation method in which polymerizable monomers of the binder resin are emulsion-polymerized, the formed dispersion liquid and a dispersion liquid of the colorant, the release agent, the charge-controlling agent as necessary, and the like are mixed, aggregated, heated, and coalesced so as to obtain toner particles; a suspension polymerization method in which polymerizable monomers for obtaining the binder resin and a solution of the colorant, the release agent, the charge-controlling agent as necessary, and the like are suspended in an aqueous solvent so as to polymerize the monomers; a dissolution suspension method in which the binder resin and a solution of the colorant, the release agent, the charge-controlling agent as necessary, and the like are suspended in an aqueous solvent so as to granulate the binder resin; or the like. In addition, the toner particles may be manufactured by a method in which the toner particles obtained by the above method are used as cores, and, furthermore, aggregated particles are attached, heated, and coalesced so as to prepare a core shell structure.

Among the above, the toner of the exemplary embodiment is preferably a toner (emulsion aggregation toner) obtained by the emulsion and aggregation method or the emulsion polymerization aggregation method.

The particle diameter of the toner particle manufactured in the above manner is preferably in a range of 2  $\mu\text{m}$  to 8  $\mu\text{m}$ , and more preferably in a range of 3  $\mu\text{m}$  to 7  $\mu\text{m}$  in terms of volume average particle diameter. When the volume average particle diameter is 2  $\mu\text{m}$  or more, since the fluidity of the toner is favorable and sufficient charging ability is imparted from the carrier, fogging in the background portion does not easily occur, and density reproducibility does not easily degrade. In

addition, when the volume average particle diameter is 8  $\mu\text{m}$  or less, the effect of improving the reproducibility, tone, and granularity of fine dots is favorable, and a high-quality image may be obtained. Meanwhile, the volume average particle diameter is measured using a measurement device, such as a COULTER MULTISIZER II (manufactured by Beckman Coulter, Inc.).

The toner particles are preferably pseudospherical from the viewpoints of improvement in the developability, transfer efficiency, and image qualities. The degree of spheroidizing of the toner particles may be expressed using the shape coefficient SF1 in the formula shown below, and the average value (average shape coefficient) of the shape coefficient SF1 of the toner particles used in the exemplary embodiment is preferably less than 145, more preferably in a range of 115 to less than 140, and still more preferably in a range of 120 to less than 140. When the average value of the shape coefficient SF1 is less than 145, favorable transfer efficiency may be obtained, and the image quality is excellent.

$$SF1 = \left| \frac{(ML)^2}{A} \times \frac{\pi}{4} \times 100 \right|$$

In the above formula, ML represents the maximum length of the respective toner particles, and A represents the projection area of the respective toner particles.

Meanwhile, the average value of the shape coefficient SF1 (average shape coefficient) is obtained by scanning the toner images of 1,000 particles at a magnification of 250 times into an image analyzer (LUZEX III, manufactured by Nireco Corporation) from an optical microscope, obtaining the SF1 values of the respective particles from the maximum lengths and the projection areas, and averaging the values.

#### Electrostatic Charge Image Developer

The electrostatic charge image developing toner of the exemplary embodiment is preferably used as an electrostatic charge image developer.

The electrostatic charge image developer of the exemplary embodiment is not particularly limited as long as the electrostatic charge image developer contains the electrostatic charge image developing toner of the exemplary embodiment, and may have an appropriate component composition according to the purpose. When the electrostatic charge image developing toner of the exemplary embodiment is singly used, a single-component electrostatic charge image developer is prepared, and, when the electrostatic charge image developing toner of the exemplary embodiment is used in combination with a carrier, a two-component electrostatic charge image developer is prepared.

When the single-component developer is used, a method in which the electrostatic charge image developing toner is friction-charged with a developing sleeve or a charging member so as to form a charged toner, and the toner is developed according to an electrostatic latent image is also applied.

In the exemplary embodiment, the developing method is not particularly specified, but the two-component developing method is preferable. In addition, when the above conditions are satisfied, the carrier is not particularly specified, and examples of the core material of the carrier include magnetic metals, such as iron, steel, nickel, and cobalt, alloys of the above and manganese, chromium, a rare earth element, or the like, magnetic oxides, such as ferrite and magnetite, and the like, but ferrite, particularly an alloy with manganese,

lithium, strontium, magnesium, or the like is preferable from the viewpoints of core material surface properties and core material resistance.

The carrier used in the exemplary embodiment preferably has a resin coated on the surface of the core material. The resin is not particularly limited, and appropriately selected according to purpose. Examples thereof include well-known resins, such as polyolefin resin, such as polyethylene and polypropylene; polyvinyl resin and polyvinylidene resin, such as polystyrene, an acrylic resin, polyacrylonitrile, polyvinyl acetate, polyvinyl alcohol, polyvinyl butyral, polyvinyl chloride, polyvinyl carbazole, polyvinyl ether, and polyvinyl ketone; vinyl chloride-vinyl acetate copolymer; styrene-acrylate copolymer; straight silicone resin including an organosiloxane bond and modification products thereof; fluorine resin, such as polytetrafluoroethylene, polyvinyl fluoride, polyvinylidene fluoride, and polychlorotrifluoroethylene; a silicone resin; polyester; polyurethane; polycarbonate; a phenol resin; amino resin, such as a urea-formaldehyde resin, a melamine resin, a benzoguanamine resin, a urea resin, and a polyamide resin; and an epoxy resin. The resin may be used singly, or two or more kinds may be jointly used. In the exemplary embodiment, among the above resins, at least the fluorine resins and/or the silicone resin are preferably used. When at least the fluorine resins and/or the silicone resin are used as the resin, the effect of preventing carrier contamination (impaction) due to the toner or the external additive is favorable, which is advantageous.

A film formed of the resin preferably has resin particles and/or conductive particles dispersed in the resin. Examples of the resin particles include thermoplastic resin particles, thermosetting resin particles, and the like. Among the above, a thermosetting resin is preferable from the viewpoint of a relatively easy increase in the hardness, and resin particles of a nitrogen-containing resin containing N atoms is preferable from the viewpoint of imparting negative chargeability to the toner. Meanwhile, the resin particles may be used singly, or two or more kinds may be jointly used. The average particle diameter of the resin particles is preferably from 0.1  $\mu\text{m}$  to 2  $\mu\text{m}$ , and more preferably from 0.2  $\mu\text{m}$  to 1  $\mu\text{m}$ . When the average particle diameter of the resin particles is 0.1  $\mu\text{m}$  or more, the dispersibility of the resin particles in the film is excellent, and, on the other hand, when the average particle diameter of the resin particles is 2  $\mu\text{m}$  or less, the resin particles do not easily fall off from the film.

Examples of the conductive particles include metal particles of gold, silver, copper, and the like, carbon black particles, furthermore, particles obtained by coating the surfaces of titanium oxide, zinc oxide, barium sulfate, aluminum borate, potassium titanate powder, or the like with tin oxide, carbon black, metals, or the like. The conductive particles may be used singly, or two or more kinds may be jointly used. Among the above, carbon black particles are preferable in terms of favorable manufacturing stability, costs, conductivity, and the like. The kind of the carbon black is not particularly limited, but carbon black having a IMP oil absorption of 50 ml/100 g to 250 ml/100 g is preferable since the manufacturing stability is excellent. The amounts of the resin, the resin particles, and the conductive particles coated on the surface of the core material are preferably 0.5% by weight to 5.0% by weight, and more preferably 0.7% by weight to 3.0% by weight.

A method of forming the film is not particularly limited, and examples thereof include a method in which a film-forming liquid including the resin particles, such as crosslinking resin particles, and/or the conductive particles, and the

resin, such as a styrene acrylic resin, a fluorine resin, a silicone resin, or the like as a matrix resin in a solvent is used.

Specific examples thereof include an immersion method in which the carrier core material is immersed in the film-forming liquid, a spray method in which the film-forming liquid is sprayed to the surface of the carrier core material, a kneader coater method in which the film-forming liquid is mixed in a state in which the carrier core material is floated using an air flow, and the solvent is removed, and the like. Among the above, in the exemplary embodiment, the kneader coater method is preferable.

The solvent used in the film-forming liquid is not particularly limited as long as the solvent may dissolve the resin as the matrix resin only, and may be selected from well-known solvents. Examples of the solvent include aromatic hydrocarbons, such as toluene and xylene; ketones, such as acetone and methyl ethyl ketone; ethers, such as tetrahydrofuran and dioxane; and the like. In a case in which the resin particles are dispersed in the film, since the resin particles and the particles as the matrix resin are uniformly dispersed in the thickness direction and the tangential direction to the carrier surface, even when the carrier is used for a long time such that the film is worn, the same surface formation may be held as before use, and favorable chargeability may be maintained for a long time with respect to the toner. In addition, in a case in which the conductive particles are dispersed in the film, since the conductive particles and the resin as the matrix resin are uniformly dispersed in the thickness direction and the tangential direction to the carrier surface, even when the carrier is used for a long time such that the film is worn, the same surface formation may be held as before use, and deterioration of the carrier is prevented for a long time. Meanwhile, in a case in which the resin particles and the conductive particles are dispersed in the film, the above effects are exhibited at the same time.

The electrical resistance of the entire magnetic carrier formed in the above manner is preferably from  $10^8 \Omega/\text{cm}^2$  to  $10^{13} \Omega/\text{cm}^2$  in a state of magnetic brush under an electric field of  $10^4 \text{ V/cm}$ . When the electrical resistance of the magnetic carrier is  $10^8 \Omega/\text{cm}^2$  or more, attachment of the carrier to the image portion on the image holding member is suppressed, and brush marks are not easily generated. On the other hand, when the electrical resistance of the magnetic carrier is  $10^{13} \Omega/\text{cm}^2$  or less, occurrence of the edge effect is suppressed, and favorable image qualities may be obtained.

Meanwhile, the electrical resistance (volume intrinsic resistance) is measured in the following manner.

Samples are mounted on the bottom electrode plate of a measurement jig which is a pair of  $20 \text{ cm}^2$  circular (steel) electrode plates that is connected to an electrometer (manufactured by Keithley Instruments Inc., trade name: KEITHLEY 610C) and a high-pressure power supply (manufactured by Fluke Corporation, trade name: FLUKE 415B) so as to form an approximately 1 mm to 3 mm-thick flat layer. Next, the upper electrode plate is placed on the samples, and then a 4 kg weight is placed on the upper electrode plate in order to remove voids between the samples. The thickness of the sample layer is measured in the current state. Next, an electric current value is measured by applying a voltage to both electrode plates, and a volume intrinsic resistance is computed based on the following formula.

$$\text{Volume intrinsic resistance} = \frac{\text{applied voltage} \times 20}{(\text{electric current value} - \text{initial electric current value}) \times \text{sample thickness}}$$

In the above formula, the initial electric current refers to an electric current value when the applied voltage is zero, and the electric current value refers to a measured electric current value.

5 The mixing ratio of the toner and the carrier of the exemplary embodiment in the two-component electrostatic charge image developer is preferably from 2 parts by weight to 10 parts by weight of the toner with respect to 100 parts by weight of the carrier. In addition, the method of preparing the 10 developer is not particularly limited, and examples thereof include a method in which a V blender is used for mixing, and the like.

#### Image Forming Method

In addition, the electrostatic charge image developer (electrostatic charge image developing toner) is used in an electrostatic charge image developing-type (electrophotography-type) image forming method.

The image forming method of the exemplary embodiment includes charging a surface of an image holding member, 20 forming an electrostatic latent image on the surface of the image holding member, developing the electrostatic latent image formed on the surface of the image holding member using a developer including a toner so as to form a toner image, and transferring the toner image to the surface of a transfer medium, and may further include fixing the toner image transferred to the surface of the transfer medium, and cleaning the electrostatic charge image developer remaining on the image holding member, in which the electrostatic charge image developing toner of the exemplary embodiment 25 or the electrostatic charge image developer of the exemplary embodiment is used as the developer.

The respective processes are an ordinary process, and described in, for example, JP-A-56-40868, JP-A-49-91231, and the like. Meanwhile, in the image forming method of the 30 exemplary embodiment, a well-known image forming apparatus, such as a copying machine or a fax machine, may be used.

Forming an electrostatic latent image is a process in which an electrostatic latent image is formed on an image holding 40 member (photoreceptor).

Developing the electrostatic latent image is a process in which the electrostatic latent image is developed using a developer layer on a developer holding member so as to form a toner image. The developer layer is not particularly limited 45 as long as the developer layer includes the electrostatic charge image developing toner of the exemplary embodiment.

Transferring the toner image is a process in which the toner image is transferred to a transfer medium. In addition, examples of the transfer medium while transferring the toner image include a recording medium, such as an intermediate 50 transfer article or paper.

While fixing the toner image, for example, the toner image transferred to a transfer paper is fixed using a heating roller fixing machine for which the temperature of the heating roller 55 is set to a certain temperature so as to form a copying image.

Cleaning the electrostatic charge image developer is a process in which the electrostatic charge image developer remaining on the image holding member is cleaned.

In addition, in the image forming method of the exemplary 60 embodiment, cleaning the electrostatic charge image developer more preferably includes removing the electrostatic charge image developer remaining on the image holding member using a cleaning blade.

A well-known recording medium may be used as the 65 recording medium, and examples thereof include paper, an OHP sheet, and the like that are used in an electrophotography-type copying machine, a printer, or the like. Preferable

examples that may be used include coated paper obtained by coating the surface of plain paper with a resin or the like, printing art paper, and the like.

The image forming method of the exemplary embodiment may further include recycling. The recycling is a process in which the electrostatic charge image developing toner collected during the cleaning of the electrostatic charge image developer is moved to the developer layer. In the image forming method including the recycling, an image forming apparatus, such as a toner recycling system-type copying machine, fax machine, or the like, is used. In addition, the image forming method may be applied to a recycle system in which the toner is collected at the same time as developing.

#### Image Forming Apparatus

The image forming apparatus of the exemplary embodiment has an image holding member, a charging unit that charges a surface of the image holding member, a latent image forming unit that forms an electrostatic latent image on the surface of the image holding member, a developing unit that develops the electrostatic latent image using a developer including the toner so as to form a toner image, and a transfer unit that transfers the toner image from the image holding member to the surface of the transfer medium, and may further include a fixing unit that fixes the toner image transferred to the surface of the transfer medium, and a cleaning unit that cleans the image holding member, in which the electrostatic charge image developing toner of the exemplary embodiment or the electrostatic charge image developer of the exemplary embodiment is used as the developer.

Meanwhile, the image forming apparatus of the exemplary embodiment is not particularly limited as long as the image forming apparatus includes at least the image holding member, the charging unit, the exposure unit, the developing unit, the transfer unit, the fixing unit, and the cleaning unit, and may also include an erasing unit and the like as necessary.

In the transfer unit, two or more times of transfer may be carried out using an intermediate transfer article. In addition, examples of the transfer medium in the transfer unit include recording medium, such as an intermediate transfer article and paper.

The image holding member and the respective units may preferably use the configuration that has been described in the respective processes of the above image forming method. Well-known units for the image forming apparatus may be used as the respective units. In addition, the image forming apparatus of the exemplary embodiment may include units, apparatuses, and the like other than the above configuration. In addition, in the image forming apparatus of the exemplary embodiment, plural units of the above-described units may be operated at the same time.

In addition, examples of the cleaning unit that cleans the electrostatic charge image developer remaining on the image holding member include a cleaning blade, a cleaning brush, and the like, and a cleaning blade is preferable.

A preferable material of the cleaning blade includes urethane rubber, neoprene rubber, silicone rubber, and the like.

Toner Cartridge, Developer Cartridge, and Process Cartridge

The toner cartridge of the exemplary embodiment is a toner cartridge including a toner containing chamber that accommodates at least the electrostatic charge image developing toner of the exemplary embodiment.

The developer cartridge of the exemplary embodiment is a developer cartridge including a developer containing chamber that accommodates at least the electrostatic charge image developer of the exemplary embodiment.

In addition, the process cartridge of the exemplary embodiment has a developing unit that develops the electrostatic latent image formed on the surface of the image holding member using the electrostatic charge image developing toner or the electrostatic charge image developer so as to form a toner image, and at least one kind selected from a group consisting of the image holding member, the charging unit for charging the surface of the image holding member, and the cleaning unit for removing the toner remaining on the surface of the image holding member, and accommodates at least the electrostatic charge image developing toner of the exemplary embodiment or the electrostatic charge image developer of the exemplary embodiment.

The toner cartridge of the exemplary embodiment is preferably detachable from the image forming apparatus. That is, in an image forming apparatus having a configuration in which the toner cartridge may be detachable, the toner cartridge of the exemplary embodiment which accommodates the toner of the exemplary embodiment is preferably used.

The developer cartridge of the exemplary embodiment is not particularly limited as long as the developer cartridge contains an electrostatic charge image developer including the electrostatic charge image developing toner of the exemplary embodiment. For example, the developer cartridge is detachable from an image forming apparatus having a developing unit, and accommodates an electrostatic charge image developer including the electrostatic charge image developing toner of the exemplary embodiment as a developer for being supplied to the developing unit.

In addition, the developer cartridge may be a cartridge accommodating a toner and a carrier, or a cartridge separately having a cartridge singly accommodating a toner and a cartridge singly accommodating a carrier.

The process cartridge of the exemplary embodiment is preferably detachable from the image forming apparatus.

In addition, the process cartridge of the exemplary embodiment may include other members, such as an erasing unit, as necessary.

The toner cartridge and the process cartridge may employ a well-known configuration, and, for example, JP-A-2008-209489, JP-A-2008-233736, and the like may be referenced.

#### EXAMPLES

Hereinafter, the exemplary embodiment will be described in detail using examples, but the examples do not limit the exemplary embodiment. Meanwhile, in the following description, "parts" refers to "parts by weight" unless otherwise described.

Method of measuring the weight average molecular weight and molecular weight distribution of the resin

The molecular weight and molecular weight distribution of the binder resin are measured under the following conditions.

An "LC-8120 GPC, SC8020 (manufactured by Tosoh Corporation) apparatus" is used for the GPC, two pieces of "TSKgel Super HM H (manufactured by Tosoh Corporation, 6.0 mmID×15 cm)" are used as the column, and tetrahydrofuran (THF) is used as an eluting solution. An experiment is carried out using an IR detecting machine under the experiment conditions of a sample concentration of 0.5%, a flow rate of 0.6 mL/min, a sample injection amount of 10  $\mu$ L, and a measurement temperature of 40°C. In addition, the standard curve is prepared from 10 samples of "polystyrene standard sample TSK standard" manufactured by Tosoh Corporation: "A500," "F1," "F10," "F80," "F380," "A2500," "F4," "F40," "F128," and "F700."

21

Volume average particle diameters of resin particles, colorant particles, and the like

The volume average particle diameters of the resin particles, the colorant particles, and the like are measured using a laser diffraction particle size distribution measurement apparatus (manufactured by Horiba, Ltd., LA700).

Method of measuring the melting point and glass transition temperature of the resin

The melting point of a crystalline polyester resin and the glass transition temperature ( $T_g$ ) of an amorphous polyester resin are obtained from the measured main maximum peak using a differential scanning calorimeter (manufactured by PerkinElmer Co., Ltd., DSC 7) based on ASTM D-34188. The melting points of indium and zinc are used for temperature correction in the detecting portion of the apparatus (DSC 7), and the melting heat of indium is used for correction of the heat amount. An aluminum pan is used for a sample, an empty pan is set for reference, and measurement is carried out at a temperature increase rate of  $10^\circ \text{C}/\text{min}$ .

Method of Measuring the Volume Average Particle Diameter of the Toner

The volume average particle diameter of the toner particles is measured using a COULTER MULTISIZER II (manufactured by Beckman Coulter, Inc.). ISOTON-II (manufactured by Beckman Coulter, Inc.) is used as an electrolytic solution.

In the measurement method, firstly, 0.5 mg to 50 mg of the measurement sample is added to a surfactant, preferably 2 ml of a 5% aqueous solution of sodium alkyl benzene sulfonate, as a dispersion agent, and the mixture is added to 100 ml to 150 ml of the electrolytic solution. The electrolytic solution having the measurement sample suspended is dispersed in an ultrasonic dispersing device for approximately 1 minute, and the particle size distribution of particles having a particle diameter in a range of  $2.0 \mu\text{m}$  to  $60 \mu\text{m}$  is measured using an aperture having an aperture radius of  $100 \mu\text{m}$  in the COULTER MULTISIZER II. The number of particles measured is set to 50,000.

For the measured particle size distribution, the cumulative distribution is drawn from the smaller diameter side in terms of weight or volume in a divided particle size range (channel), and the particle diameter corresponding to 50% cumulative value is defined as the weight average particle diameter or the volume average particle diameter.

Method of Obtaining the Shape Coefficient

The shape coefficient SF1 is obtained from the following formula.

$$SF1 = 100 \pi \times (ML)^2 / (4 \times A)$$

Here, ML represents the maximum length of the particles, and A represents the projection area of the particles. The maximum length and projection area of the particles are obtained by observing particles sampled on a glass slide using an optical microscope, scanning into an image analyzer (LUZEX III, manufactured by Nireco Corporation) through a video camera, and carrying out an image analysis. The number of particles sampled at this time is 100 or more, and the shape coefficient shown in the formula is obtained using the average value.

Preparation of the Toner Particles

Preparation of the Respective Dispersion Liquids

Preparation of Crystalline Polyester Resin Particle Dispersion Liquid 1

After 260 parts by weight of 1,12-dodecanedicarboxylic acid, 165 parts by weight of 1,10-decanediol, and 0.035 part by weight of tetrabutoxy titanate as a catalyst are put in a heated and dried three-necked flask, the air in the container is depressurized through a depressurization operation, further-

22

more, an inert atmosphere is formed using nitrogen gas, and reflux is carried out at  $180^\circ \text{C}$ . for 6 hours through mechanical stirring. After that, the temperature is slowly increased up to  $220^\circ \text{C}$ . through distillation under reduced pressure, the mixture is stirred for 2 to 3 hours, the distillation under reduced pressure is stopped when a viscous state is formed, and the mixture is cooled in the air, thereby obtaining a crystalline polyester resin 1.

The weight average molecular weight ( $M_w$ ) of the obtained crystalline polyester resin 1 which is measured by the above method is 12,000. In addition, the melting point of the obtained crystalline polyester resin 1 is measured by the above measurement method using a differential scanning calorimeter (DSC), and is found to be  $72^\circ \text{C}$ .

Next, 180 parts by weight of the crystalline polyester resin 1 and 580 parts by weight of deionized water are put in a stainless beaker, and heated to  $95^\circ \text{C}$ . by placing the beaker in a warm bath. The mixture is stirred at 8,000 rpm using a homogenizer (manufactured by IKA Laboratory Technology, ULTRA-TURRAX T50) when the crystalline polyester resin 1 is melted, and, at the same time, diluted ammonia water is added so as to adjust the pH to 7.0. Next, while 20 parts by weight of an aqueous solution having 0.8 part by weight of an anionic surfactant (manufactured by Dai-ichi Kogyo Seiyaku Co., Ltd., NEOGEN R) diluted therein is added dropwise, emulsion dispersion is carried out, thereby preparing a crystalline polyester resin particle dispersion liquid 1 (resin particle concentration: 12.5% by weight) having a volume average particle diameter of  $0.24 \mu\text{m}$ .

Preparation of Amorphous Polyester Resin Particle Dispersion Liquid 1

After 73 parts by weight of dimethyl adipate, 182 parts by weight of dimethyl terephthalate, 217 parts by weight of bisphenol A ethylene oxide adduct, 41 parts by weight of ethylene glycol, and 0.038 part by weight of tetrabutoxy titanate as a catalyst are put in a heated and dried two-necked flask, nitrogen gas is put into the container so as to maintain an inert atmosphere, the mixture is heated while being stirred, then, a condensation copolymerization reaction is caused at  $160^\circ \text{C}$ . for approximately 7 hours, then, the temperature is increased up to  $220^\circ \text{C}$ . while the pressure is slowly decreased up to 10 Torr, and the atmosphere is held for 3.5 hours. Once the pressure returns to an ordinary pressure, 9 parts by weight of trimellitic anhydride is added, the pressure is again slowly reduced up to 10 Torr, and the atmosphere is held for 1 hour, thereby synthesizing an amorphous polyester resin 1.

The glass transition temperature of the obtained amorphous polyester resin 1 is measured by the above measurement method using a differential scanning calorimeter (DSC), and is found to be  $58^\circ \text{C}$ . The molecular weight of the obtained amorphous polyester resin 1 is measured by the above measurement method using a GPC, and the weight average molecular weight ( $M_w$ ) is 11,000.

Next, 115 parts by weight of the amorphous polyester resin 1, 180 parts by weight of deionized water, and 5 parts by weight of an anionic surfactant (manufactured by Dai-ichi Kogyo Seiyaku Co., Ltd., NEOGEN R) are mixed, heated at  $120^\circ \text{C}$ ., then, sufficiently dispersed using a homogenizer (manufactured by IKA Laboratory Technology, ULTRA-TURRAX T50), and then a dispersion treatment is carried out for 1 hour using a pressure ejection-type Gaulin homogenizer, thereby preparing an amorphous polyester resin particle dispersion liquid 1 (resin particle concentration: 40% by weight).

23

Preparation of Styrene Acrylic Resin Dispersion Liquid 1  
Oil Layer  
Styrene (manufactured by Wako Pure Chemical Industries, Ltd.): 32 parts by weight  
n-butyl acrylate (manufactured by Wako Pure Chemical Industries, Ltd.): 8 parts by weight  
 $\beta$ -carboethoxy acrylate (manufactured by Rhodia Nicca): 1.2 parts by weight  
Dodecanethiol (manufactured by Wako Pure Chemical Industries, Ltd.): 0.5 part by weight

Aqueous Layer 1  
Ion exchange water: 17.0 parts by weight  
Anionic surfactant (manufactured by Rhodia Japan): 0.50 part by weight

Aqueous Layer 2  
Ion exchange water: 40 parts by weight Anionic surfactant (manufactured by Rhodia Japan): 0.06 part by weight

Ammonium persulfate (manufactured by Wako Pure Chemical Industries, Ltd.): 0.4 part by weight

The oil layer components and the components of the aqueous layer 1 are put in a flask, stirred, and mixed so as to prepare a monomer emulsion dispersion liquid. The components of the aqueous layer 2 are injected into a reaction container, the inside of the container is sufficiently substituted with nitrogen, and the mixture is heated in an oil bath under stirring so that the temperature of the reaction system reaches 75°C.

The monomer emulsion dispersion liquid is slowly added dropwise to the reaction container over 3 hours so as to carry out emulsion polymerization. After the dropwise addition, polymerization is continued at 75°C., and the polymerization is completed after 3 hours, thereby obtaining a styrene acrylic resin dispersion liquid.

The volume average particle diameter of the resin particles in the obtained styrene acrylic resin dispersion liquid is 330 nm, and the weight average molecular weight (Mw) is measured by the above method, and is found to be 12,500. In addition, the glass transition temperature is measured by the above measurement method using a differential scanning calorimeter (DSC), and is found to be 52°C.

#### Preparation of Colorant Dispersion Liquid

After 100 parts by weight of a cyan pigment (manufactured by Dainichiseika Color & Chemicals Mfg. Co., Ltd., Pigment Blue 15:3 (copper phthalocyanine), 15 parts by weight of an anionic surfactant (manufactured by Dai-ichi Kogyo Seiyaku Co., Ltd., NEOGEN R), and 300 parts by weight of ion exchange water are mixed, dispersed for 10 minutes using a homogenizer (manufactured by IKA Laboratory Technology, ULTRA-TURRAX T50), and then subjected to a circulation-type ultrasonic dispersion machine (manufactured by Nissei Corporation, RUS 600TCVP), thereby obtaining a colorant dispersion liquid.

The volume average particle diameter of the colorant (cyan pigment) in the obtained colorant dispersion liquid is measured by the above measurement method using a laser diffraction particle size measuring machine, and is found to be 0.17  $\mu$ m. In addition, the solid content proportion of the cyan colorant dispersion liquid is 24% by weight.

#### Preparation of Release Agent Dispersion Liquid

After 95 parts by weight of Fischer-Tropsch wax FNP92 (melting point: 92°C., manufactured by Nippon Seiro Co., Ltd.) 3.6 parts by weight of an anionic surfactant (manufactured by Dai-ichi Kogyo Seiyaku Co., Ltd., NEOGEN R), and 360 parts by weight of ion exchange water are mixed, heated to 100°C., and sufficiently dispersed using a homogenizer (manufactured by TKA Laboratory Technology, ULTRA-TURRAX T50), a dispersion treatment is carried out using a

24

pressure ejection-type Gaulin homogenizer, thereby obtaining a release agent dispersion liquid.

The volume average particle diameter of the release agent in the obtained release agent dispersion liquid is measured by the above measurement method using a laser diffraction particle size measuring machine, and is found to be 0.24  $\mu$ m. In addition, the solid content proportion of the release agent dispersion liquid is 20% by weight.

#### Preparation of Toner Particles 1

10 104.4 parts by weight of the crystalline polyester resin particle dispersion liquid 1, 336.1 parts by weight of the amorphous polyester resin particle dispersion liquid 1, 45.4 parts by weight of the colorant dispersion liquid, 115.3 parts by weight of the release agent dispersion liquid, and 484 parts by weight of deionized water are put in a round stainless flask, sufficiently mixed using an ULTRA-TURRAX T50, and dispersed. Next, 0.37 part by weight of polyaluminum chloride is added to the mixture, and the mixture is continuously subjected to a dispersion operation in the ULTRA-TURRAX. 15 Furthermore, the mixture is heated up to 52°C. while stirring the flask in a heating oil bath. After the mixture is held at 52°C. for 3 hours, 175 parts by weight of the amorphous polyester resin particle dispersion liquid 1 is slowly added to the mixture. After that, the pH inside the system is adjusted to 8.5 20 using a 0.5 N sodium hydroxide aqueous solution, then the stainless steel flask is sealed, heated up to 90°C. while continuously stirred using a magnetic seal, and held for 3 hours. After completion of the reaction, the mixture is cooled, filtered, sufficiently washed using ion exchange water, and then 25 solid and liquid are separated through Nutsche-type suction filtration. The mixture is again dispersed in 3 L of ion exchange water at 30°C., stirred at 300 rpm for 15 minutes, and washed. The above processes are repeated 5 more times, washing is ended when the pH of the filtrate becomes 6.85, 30 the electrical conductivity becomes 8.2  $\mu$ S/cm, and the surface tension becomes 7.05 Nm, solid and liquid are separated through Nutsche-type suction filtration using No. 5A filtering paper, and then vacuum drying is carried out for 12 hours, thereby obtaining toner particles 1.

35 40 The glass transition temperature of the obtained toner particles 1 is measured by the above method, and is found to be 54.0°C. The volume average particle diameter of the toner particles 1 is measured by the above measurement method, and is found to be 5.8  $\mu$ m. In addition, the average degree of circularity of the toner particles 1 is measured by the above measurement method, and is found to be 0.959.

#### Preparation of Toner Particles 2

45 Styrene acrylic resin dispersion liquid 1: 70 parts by weight  
Colorant dispersion liquid: 14 parts by weight  
Release agent dispersion liquid: 22 parts by weight  
Polyaluminum chloride: 0.14 part by weight

The above components are sufficiently mixed and dispersed in a round stainless steel flask using an ULTRA-TURRAX T50. Next, 0.32 part by weight of polyaluminum 55 chloride is added to the mixture, and a dispersion operation is continued using the ULTRA-TURRAX. The mixture is heated to 47°C. while the flask is stirred in a heating oil bath. After the mixture is held at 47°C. for 60 minutes, 30 parts by weight of the binder resin dispersion liquid is slowly added to the mixture.

60 After that, the phi inside the system is adjusted to 6.0 using 0.5 mol/L of a sodium hydroxide aqueous solution, then, the stainless steel flask is sealed, the mixture is heated to 96°C. while stirring is continued using a magnetic seal, and held for 3.5 hours. After completion of the reaction, the mixture is cooled, filtered, sufficiently washed using ion exchange water, and then solid and liquid are separated through Nut-

## 25

sche-type suction filtration. Furthermore, the mixture is again dispersed in 3 L of ion exchange water at 40°C, stirred at 300 rpm for 15 minutes and washed.

The above processes are repeated 5 more times, and solid and liquid are separated through Nutsche-type suction filtration using No. 5A filtering paper when the pH of the filtrate becomes 7.01, the electrical conductivity becomes 9.7  $\mu$ S/cm, and the surface tension becomes 71.2 Nm. Next, vacuum drying is continued for 12 hours, thereby manufacturing toner particles 2.

The volume average particle diameter of the obtained toner particles 2 is measured by the above measurement method, and is found to be 5.7  $\mu$ m. In addition, the average degree of circularity of the toner particles 2 is measured by the above measurement method, and is found to be 0.957.

## Preparation of Toner Particles 3

A mixture of 100 parts of a styrene-butyl acrylate copolymer (weight average molecular weight Mw=150,000, copolymerization ratio 80:20), 5 parts of carbon black (MOGUL L, manufactured by Cabot Corporation), and 6 parts of carnauba wax is kneaded using an extruder, pulverized using a jet mill, then, a spheroidizing treatment using warm air is carried out using a KRYPTON (manufactured by Kawasaki Heavy Industries Ltd.), and the mixture is classified using a wind-power classifier, thereby obtaining toner particles 3 having a particle diameter of 6.2  $\mu$ m.

## External Additive

Inorganic particles having an aliphatic alcohol present on the surface thereof as described in Examples 1 to 8 and Comparative Examples 1 to 3 in Table 1 are prepared by treating silica ( $\text{SiO}_2$ ) particles or titanium oxide particles using the aliphatic alcohol described in Table 1 in an amount corresponding to 0.50% by weight or 0.20% by weight. The inorganic particles (2% by weight) having the aliphatic alcohol present on the surface thereof is added to toner particles, and mixed using a Henschel mixer, thereby manufacturing an externally added toner.

## Preparation of Treatment External Additive 1

Hydrophobic fumed silica R8200 (average particle diameter 12 nm, manufactured by Nippon Aerosil Co., Ltd.) (10 parts by weight) and 1-decanol (manufactured by Tokyo Chemical Industry Co., Ltd.) (2.5 parts by weight) are mixed using a sample mill, thereby obtaining a treatment external additive 1.

## Preparation of Treatment External Additive 2

Hydrophobic fumed silica 88200 (average particle diameter 12 nm, manufactured by Nippon Aerosil Co., Ltd.) (10 parts by weight) and 2-pentanol (manufactured by Tokyo Chemical Industry Co., Ltd.) (2.5 parts by weight) are mixed using a sample mill, thereby obtaining a treatment external additive 2.

## Preparation of Treatment External Additive 3

Hydrophobic fumed silica 88200 (average particle diameter 12 nm, manufactured by Nippon Aerosil Co., Ltd.) (10 parts by weight) and isostearyl alcohol EX (component: isostearyl alcohol, manufactured by Kokyu Alcohol Kogyo Co., Ltd.) (2.5 parts by weight) are mixed using a sample mill, thereby obtaining a treatment external additive 3.

## Preparation of Treatment External Additive 4

Hydrophobic fumed silica R8200 (average particle diameter 12 nm, manufactured by Nippon Aerosil Co., Ltd.) (10 parts by weight) and isostearyl alcohol EX (component: isostearyl alcohol, manufactured by Kokyu Alcohol Kogyo Co., Ltd.) (1.0 part by weight) are mixed using a sample mill, thereby obtaining a treatment external additive 4.

## 26

## Preparation of Treatment External Additive 5

Hydrophobic titanium oxide JMT-150AO (average particle diameter 15 nm, manufactured by Tayca Corporation) (10 parts by weight) and isostearyl alcohol EX (component: isostearyl alcohol, manufactured by Kokyu Alcohol Kogyo Co., Ltd.) (2.5 parts by weight) are mixed using a sample mill, thereby obtaining a treatment external additive 5.

## Preparation of Treatment External Additive 6

Hydrophobic fumed silica R8200 (average particle diameter 12 nm, manufactured by Nippon Aerosil Co., Ltd.) (10 parts by weight) and 1-decanol (manufactured by Tokyo Chemical Industry Co., Ltd.) (10 parts by weight) are mixed using a sample mill, thereby obtaining a treatment external additive 6.

## 15 Preparation of Treatment External Additive 7

Hydrophobic fumed silica R8200 (average particle diameter 12 nm, manufactured by Nippon Aerosil Co., Ltd.) (10 parts by weight) and dimethyl silicone oil KF-96-50cs (manufactured by Shin-Etsu Chemical Co., Ltd.) (2.5 parts by weight) are mixed using a sample mill, thereby obtaining a treatment external additive 7.

## Preparation of Treatment External Additive 8

Hydrophobic fumed silica R8200 (average particle diameter 12 nm, manufactured by Nippon Aerosil Co., Ltd.) (10 parts by weight) and stearyl alcohol (manufactured by Wako Pure Chemical Industries, Ltd.) (2.5 parts by weight) are mixed using a sample mill, thereby obtaining a treatment external additive 8.

## Preparation of Treatment External Additive 9

Hydrophobic fumed silica 88200 (average particle diameter 12 nm, manufactured by Nippon Aerosil Co., Ltd.) (10 parts by weight) and 1-butanol (manufactured by Tokyo Chemical Industry Co., Ltd.) (2.5 parts by weight) are mixed using a sample mill, thereby obtaining a treatment external additive 9.

## Example 1

## Preparation of Externally Added Toner 1

The treatment external additive 1 (2 parts by weight) is added to 100 parts by weight of the toner particles 1, and the resultant is blended using a sample mill, thereby obtaining an externally added toner 1.

## 45 Preparation of Developer 1

The externally added toner 1 is weighed so that the toner concentration becomes 5% by weight with respect to a ferrite carrier which is coated with 1% by weight of polymethyl methacrylate (manufactured by Soken Chemical & Engineering Co., Ltd.) and has a volume average particle diameter of 50 stirred, and mixed using a V blender for 30 minutes, thereby preparing a developer 1.

The following image output test and cleaning property test are carried out using the obtained developer 1.

55 The obtained results are summarized and shown in Table 1.

Image Output Test (Electric Charge Leakage-Induced Ground Fogging)

A test of outputting 30,000 sheets of images over 2 days using a machine obtained by modifying DocuCenterColor 60400 (manufactured by Fuji Xerox Co., Ltd.), A4-sized plain paper (manufactured by Fuji Xerox Co., Ltd., C2 paper), and 5% of the Imaging Society of Japan's test chart No. 8 under a high-humidity environment of 30°C. and 88% is carried out. 20,000 sheets are continuously outputted on the first day, the Imaging Society of Japan's test chart No. 1 is outputted with one operation next morning, and then, furthermore, 10,000 sheets are continuously outputted for one day. After 30,000

27

sheets in total are outputted, the Imaging Society of Japan's test chart No. 1 is outputted with one operation next morning, and image qualities are evaluated. In the evaluation, A to C is set to an acceptable range.

A: No fogging is observed on the image, there is no problem with image quality, and no contamination in the actual machine is observed.

B: No fogging is observed on the image, but contamination in the actual machine is slightly observed.

C: Fogging is slightly observed on the image, and contamination in the actual machine is observed.

D: Fogging and deterioration of the reproducibility of fine lines are observed on the image, and contamination in the actual machine is observed.

Cleaning Properties (Filming-Induced Cleaning Properties)

A test of outputting 30,000 sheets of images using a machine obtained by modifying DocuCenterColor 400 (manufactured by Fuji Xerox Co., Ltd.), A4-sized plain paper (manufactured by Fuji Xerox Co., Ltd., C2 paper), and 5% of the Imaging Society of Japan's test chart No. 8 under a low-humidity environment of 20° C. and 15% is carried out. For every 10,000 sheets, the photoreceptor is removed, and the photoreceptor surface and the outputted image surface are visually observed. The evaluation standards are as follows, and A and B is set to an allowable range. Meanwhile, for samples evaluated to be D, the test is stopped at that stage. At a point in time when 20,000 sheets are completed, samples evaluated to be B or better are considered to be excellent in terms of cleaning properties as the toner according to the exemplary embodiment.

A: Neither attachment of foreign substances on the photoreceptor nor toner contamination on the image could be observed visually.

B: Attachment of foreign substances is observed on the photoreceptor, but toner contamination is not observed on the image.

C: Attachment of foreign substances is observed on the photoreceptor, and slight toner contamination is observed on the image.

D: Toner contamination is observed on the entire surface of the photoreceptor.

### Example 2

#### Preparation of Externally Added Toner 2

The treatment external additive 2 (2 parts by weight) is added to 100 parts by weight of the toner particles 1, and blended using a sample mill, thereby obtaining an externally added toner 2.

#### Preparation of Developer 2

A developer 2 is obtained through the same operation as for the preparation of the developer 1 except that the externally added toner 2 is used instead of the externally added toner 1.

The same test as in Example 1 is carried out using the obtained developer 2.

### Example 3

#### Preparation of Externally Added Toner 3

The treatment external additive 3 (2 parts by weight) is added to 100 parts by weight of the toner particles 1, and blended using a sample mill, thereby obtaining an externally added toner 3.

28

#### Preparation of Developer 3

A developer 3 is obtained through the same operation as for the preparation of the developer 1 except that the externally added toner 3 is used instead of the externally added toner 1.

The same test as in Example 1 is carried out using the obtained developer 3.

### Example 4

#### Preparation of Externally Added Toner 4

The treatment external additive 4 (2 parts by weight) is added to 100 parts by weight of the toner particles 1, and blended using a sample mill, thereby obtaining an externally added toner 4.

#### Preparation of Developer 4

A developer 4 is obtained through the same operation as for the preparation of the developer 1 except that the externally added toner 4 is used instead of the externally added toner 1.

The same test as in Example 1 is carried out using the obtained developer 4.

### Example 5

#### Preparation of Externally Added Toner 5

The treatment external additive 5 (2 parts by weight) is added to 100 parts by weight of the toner particles 1, and blended using a sample mill, thereby obtaining an externally added toner 5.

#### Preparation of Developer 5

A developer 5 is obtained through the same operation as for the preparation of the developer 1 except that the externally added toner 5 is used instead of the externally added toner 1.

The same test as in Example 1 is carried out using the obtained developer 5.

### Example 6

#### Preparation of Externally Added Toner 6

The treatment external additive 1 (2 parts by weight) is added to 100 parts by weight of the toner particles 2, and blended using a sample mill, thereby obtaining an externally added toner 6.

#### Preparation of Developer 6

A developer 6 is obtained through the same operation as for the preparation of the developer 1 except that the externally added toner 6 is used instead of the externally added toner 1.

The same test as in Example 1 is carried out using the obtained developer 6.

### Example 7

#### Preparation of Externally Added Toner 7

The treatment external additive 1 (2 parts by weight) is added to 100 parts by weight of the toner particles 3, and blended using a sample mill, thereby obtaining an externally added toner 7.

#### Preparation of Developer 7

A developer 7 is obtained through the same operation as for the preparation of the developer 1 except that the externally added toner 7 is used instead of the externally added toner 1.

The same test as in Example 1 is carried out using the obtained developer 7.

## Preparation of Externally Added Toner 8

The treatment external additive 6 (4 parts by weight) is added to 100 parts by weight of the toner particles 1, and blended using a sample mill, thereby obtaining an externally added toner 8.

## Preparation of Developer 8

A developer 8 is obtained through the same operation as for the preparation of the developer 1 except that the externally added toner 8 is used instead of the externally added toner 1.

The same test as in Example 1 is carried out using the obtained developer 8.

## Comparative Example 1

## Preparation of Externally Added Toner 9

The treatment external additive 7 (2 parts by weight) is added to 100 parts by weight of the toner particles 1, and blended using a sample mill, thereby obtaining an externally added toner 9.

## Preparation of Developer 9

A developer 9 is obtained through the same operation as for the preparation of the developer 1 except that the externally added toner 9 is used instead of the externally added toner 1.

The same test as in Example 1 is carried out using the obtained developer 9.

## Preparation of Externally Added Toner 10

5 The treatment external additive 8 (2 parts by weight) is added to 100 parts by weight of the toner particles 1, and blended using a sample mill, thereby obtaining an externally added toner 10.

## Preparation of Developer 10

10 A developer 10 is obtained through the same operation as for the preparation of the developer 1 except that the externally added toner 10 is used instead of the externally added toner 1.

15 The same test as in Example 1 is carried out using the obtained developer 10.

## Comparative Example 3

## Preparation of Externally Added Toner 11

20 The treatment external additive 9 (2 parts by weight) is added to 100 parts by weight of the toner particles 1, and blended using a sample mill, thereby obtaining an externally added toner 11.

## Preparation of Developer 11

25 A developer 11 is obtained through the same operation as for the preparation of the developer 1 except that the externally added toner 11 is used instead of the externally added toner 1.

30 The same test as in Example 1 is carried out using the obtained developer 11.

TABLE 1

|                       | Toner particle   | (inorganic particle) | External additive  | Aliphatic alcohol |                                    | Treatment       | Filming-induced | Charge leakage-induced |
|-----------------------|------------------|----------------------|--------------------|-------------------|------------------------------------|-----------------|-----------------|------------------------|
|                       |                  |                      |                    | Chemical          | Number of carbon atoms             |                 |                 |                        |
| Example 1             | Toner particle 1 | Silica               | 1-decanol          | C10               | 5° C. to 7° C.<br>straight-chain   | 0.50% by weight | A               | A                      |
| Example 2             | Toner particle 1 | Silica               | 2-pentanol         | C5                | -50° C.<br>straight-chain          | 0.50% by weight | B               | A                      |
| Example 3             | Toner particle 1 | Silica               | Isostearyl alcohol | C18               | 20° C. or lower<br>branched        | 0.50% by weight | A               | A                      |
| Example 4             | Toner particle 1 | Silica               | Isostearyl alcohol | C18               | 20° C. or lower<br>branched        | 0.20% by weight | B               | A                      |
| Example 5             | Toner particle 1 | Titanium oxide       | Isostearyl alcohol | C18               | 20° C. or lower<br>branched        | 0.50% by weight | A               | B                      |
| Example 6             | Toner particle 2 | Silica               | 1-decanol          | C10               | 5° C. to 7° C.<br>straight-chain   | 0.50% by weight | A               | A                      |
| Example 7             | Toner particle 3 | Silica               | 1-decanol          | C10               | 5° C. to 7° C.<br>straight-chain   | 0.50% by weight | A               | A                      |
| Example 8             | Toner particle 1 | Silica               | 1-decanol          | C10               | 5° C. to 7° C.<br>straight-chain   | 4.0% by weight  | A               | B                      |
| Comparative example 1 | Toner particle 1 | Silica               | (silicone oil)     | —                 | —                                  | 0.50% by weight | A               | D                      |
| Comparative example 2 | Toner particle 1 | Silica               | Stearyl alcohol    | C18               | 47° C. to 53° C.<br>straight-chain | 0.50% by weight | A               | D                      |
| Comparative example 3 | Toner particle 1 | Silica               | 1-butanol          | C4                | -90° C.<br>straight-chain          | 0.50% by weight | C               | A                      |

## 31

The foregoing description of the exemplary embodiments of the present invention has been provided for the purposes of illustration and description. It is not intended to be exhaustive or to limit the invention to the precise forms disclosed. Obviously, many modifications and variations will be apparent to practitioners skilled in the art. The embodiments were chosen and described in order to best explain the principles of the invention and its practical applications, thereby enabling others skilled in the art to understand the invention for various embodiments and with the various modifications as are suited to the particular use contemplated. It is intended that the scope of the invention be defined by the following claims and their equivalents.

What is claimed is:

1. An electrostatic charge image developing toner comprising:  
toner particles that contain a colorant, a binder resin and a release agent; and  
an external additive,  
wherein the external additive contains inorganic particles including an aliphatic alcohol physically adsorbed to the surfaces thereof, the aliphatic alcohol being selected from the group consisting of 1-pentanol, 2-pentanol, 1-hexanol, 2-hexanol, 1-octanol, isooctyl alcohol, 2-ethylhexanol, 1-nonal, 1-decanol, cyclopentanol, and cyclooctanol.
2. The electrostatic charge image developing toner according to claim 1, wherein a content of the aliphatic alcohol is in a range of 0.16% by weight to 5% by weight of a total amount of the electrostatic charge image developing toner.
3. The electrostatic charge image developing toner according to claim 1, wherein 80% by area or more of the surfaces of the inorganic particles are coated with the aliphatic alcohol.
4. The electrostatic charge image developing toner according to claim 1, wherein a volume average primary particle diameter of the inorganic particles is in a range of 7 nm to 300 nm.

## 32

5. The electrostatic charge image developing toner according to claim 1, wherein a volume average primary particle diameter of the inorganic particles is in a range of 10 nm to 200 nm.
6. The electrostatic charge image developing toner according to claim 1, wherein a content of the inorganic particles including the aliphatic alcohol physically adsorbed to the surfaces thereof is in a range of 0.3% by weight to 10% by weight of a total weight of the toner.
7. The electrostatic charge image developing toner according to claim 1, wherein the toner particles contain a crystalline polyester resin in a range of 2% by weight to 30% by weight of the toner particles.
8. An electrostatic charge image developer comprising  
the toner according to claim 1; and  
a carrier.
9. A toner cartridge comprising:  
a toner containing chamber that contains the electrostatic charge image developing toner according to claim 1.
10. A developer cartridge comprising:  
a developer containing chamber that contains the electrostatic charge image developer according to claim 8.
11. A process cartridge for an image forming apparatus comprising:  
a developer holding member that holds and transports an electrostatic charge image developer,  
wherein the developer is the electrostatic charge image developer according to claim 8.
12. An image forming method comprising:  
charging a surface of an image holding member;  
forming an electrostatic latent image on the surface of the image holding member;  
developing the electrostatic latent image formed on the surface of the image holding member using a developer so as to form a toner image; and  
transferring the toner image to a recording medium,  
wherein the developer is the electrostatic charge image developer according to claim 8.

\* \* \* \* \*